

## UNITED STATES PATENT OFFICE

2,301,452

## PULP COMPOSITION AND PAPER

Joseph E. Plumstead, Wilmington, Del., assignor,  
by mesne assignments, to West Virginia Pulp  
& Paper Company, New York, N. Y., a corpora-  
tion of Delaware

No Drawing. Original application September 4,  
1931, Serial No. 561,241. Divided and this ap-  
plication June 29, 1940, Serial No. 343,095

9 Claims.

(Cl. 92—21)

This invention relates to an improved pulp composition and to paper formed therefrom. The present application is a division of my copending application Ser. No. 561,241 filed September 4, 1931, now Patent No. 2,235,531 granted March 18, 1941. In said parent case there are disclosed and claimed methods of producing certain pigment or filler materials.

The invention embraced by the present application relates to a pulp mixture containing mechanical or ground wood pulp and a substance which serves both as a filler and as an age deterrent.

Paper containing any substantial amount of mechanical or ground wood pulp has been found ordinarily to deteriorate rapidly with age. However, certain substances such as sulfites of alkaline earth metals, and particularly calcium sulfite, have been found to have an age deterrent effect upon such papers when embodied therein as a filler. Calcium sulfite may be produced in a finely divided state and of a high white color so as to render it most suitable as a filler and, due to its reducing action or the like, it tends to prevent the yellowing, due to age and exposure to air and sunlight, of paper containing it. Thus, when added as a filler to paper formed from or containing mechanical wood pulp, it not only enhances the original whiteness of the paper but it tends to preserve such whiteness.

Other features and advantages of the invention will appear from the detailed description of the same which will now be given.

For a full description of various methods and forms of apparatus by which age deterrent fillers of the types contemplated by the present invention may be produced, reference may be had to said parent Patent No. 2,235,531. These fillers are particularly valuable for paper made from mechanical or ground wood pulp. The reducing action of the calcium sulfite, for example, together with its naturally white color tends to produce a whiter paper from mechanical wood pulp and also tends to prevent the yellowing of such paper due to age and exposure to air and sunlight.

The products resulting from my process and which are particularly adapted for use as age deterring paper fillers are calcium sulfite and magnesium sulfite. Therefore, magnesium may be read into the specification and claims where calcium is specified, it being understood that calcium or an equivalent substance is intended, and that the claims are not to be restricted to calcium.

In the use of the improved pigment or filler in the production of paper, it may be added to the 55

pulp in any convenient and known manner and at any point, as in the beater, for example. The quantity may vary with the character of the paper being produced and the purposes to which it is to be put; thus, the improved filler and age deterrent may be used in any amount customary in connection with other fillers.

I claim:

1. As an article of manufacture a sheet of paper formed at least in part of mechanical wood pulp and containing calcium sulfite as an age deterrent filler.
2. A composition comprising mechanical wood pulp having calcium sulfite as an age deterrent filler distributed therethrough.
3. As an article of manufacture a sheet of paper formed at least in part of mechanical wood pulp and containing at least one sulfite of the group consisting of calcium sulfite and magnesium sulfite as an age deterrent filler.
4. A composition comprising mechanical wood pulp having at least one sulfite of the group consisting of calcium sulfite and magnesium sulfite as an age deterrent filler distributed therethrough.
5. As an article of manufacture a sheet of paper formed at least in part of mechanical wood pulp and having distributed therethrough an age deterrent filler selected from the group consisting of calcium and magnesium sulfites.
6. A composition comprising mechanical wood pulp having thoroughly inter-mixed therewith an age deterrent filler selected from the group consisting of calcium and magnesium sulfites.
7. A method of deterring the aging of paper containing mechanical wood pulp which comprises intermixing with the pulp prior to formation of paper therefrom a finely divided filler including calcium sulfite as an age deterrent.
8. A method of deterring the aging of paper containing mechanical wood pulp which comprises intermixing with the pulp prior to formation of paper therefrom a finely divided filler including at least one sulfite of the group consisting of calcium sulfite and magnesium sulfite as an age deterrent.
9. A method of deterring the aging of paper containing mechanical wood pulp which comprises introducing between the fibers thereof a finely divided filler including at least one sulfite of the group consisting of calcium sulfite and magnesium sulfite as an age deterrent.

JOSEPH E. PLUMSTEAD.